

# UNITED STATES PATENT OFFICE.

WILLIAM S. CHANDLER, OF JACKSON, MICHIGAN.

## FIRE AND WATER PROOF PAINT.

SPECIFICATION forming part of Letters Patent No. 288,621, dated November 20, 1883.

Application filed September 10, 1883. (No specimens.)

*To all whom it may concern:*

Be it known that I, WILLIAM S. CHANDLER, of the city of Jackson, in the county of Jackson, in the State of Michigan, have invented a new, useful, and important improvement upon the composition known as "fire and water proof paint," of which the following specification is a full, clear, and exact description.

10 The paint or cement herein described is specially intended for coating roofs; but it is equally adapted to the coating of walls of houses or other surfaces where, as in cellars, it is desirable to exclude all dampness.

15 The ingredients of this paint or cement consist of and are combined in the following proportions, namely: one barrel of coal-tar, forty pounds of iron-clad paint, forty pounds of sulphur, twenty pounds of Venetian red, fifteen 20 pounds of fine table-salt, ten pounds of ground alum, ten pounds of litharge, ten pounds of dry asphaltum, and twenty pounds of rosin. These ingredients are thoroughly mixed by agitation or other means. The cement is then 25 ready to be applied by a brush in the usual manner.

The iron-clad paint is made as follows: To fifty pounds of powdered iron ore is added one and one-half gallons of linseed-oil, and

the ore is ground until the ore and oil become 30 thoroughly mixed, or of the consistence of white-lead putty, when the mixture is converted into paint by adding four gallons more of the linseed-oil.

To give body to the foregoing compound, I 35 combine the tar, iron, sulphur, and Venetian red. To secure fire-proof in connection with water-proof qualities, I combine the salt, alum, and sulphur with the tar, as aforesaid. To secure a perfect finish, I add the rosin given; 40 and to secure an early hardening and to hasten the drying process, I combine the litharge and dry asphaltum.

Having thus described my invention, I claim as new and desire to secure by Letters Patent— 45

A fire and water proof paint made from coal-tar, iron-clad paint, sulphur, Venetian red, salt, alum, litharge, asphaltum, and rosin, in the manner and proportions substantially as herein set forth.

In testimony that I claim the foregoing as my own I have hereunto affixed my signature in the presence of two witnesses.

WILLIAM S. CHANDLER.

In presence of—

HORACE A. MILLS,  
P. J. DELEHANTY.